

# UNITED STATES PATENT OFFICE.

WILLIAM G. LINDSAY, OF CALDWELL, NEW JERSEY, ASSIGNOR TO THE CELLULOID COMPANY, OF NEW YORK, N. Y., A CORPORATION OF NEW JERSEY.

## PROCESS OF MAKING ACETYL-CELLULOSE PLASTICS.

1,216,581.

Specification of Letters Patent. Patented Feb. 20, 1917.

No Drawing.

Application filed November 27, 1911. Serial No. 662,747.

To all whom it may concern:

Be it known that I, WILLIAM G. LINDSAY, a citizen of the United States, residing in Caldwell, county of Essex, State of New Jersey, have invented certain new and useful Improvements in Processes of Making Acetyl-Cellulose Plastics, of which the following is a specification.

The various compositions to which the present invention relates are employed in the arts, generally as imitations of natural substances, sometimes in their original finished form with or without incorporated colors and other inert substances, and sometimes as films which are used for photographic and other purposes.

Although the final or useful form of the different compounds of acetyl cellulose is that of a solid material, the different processes of conversion into this final solid form involve, as is well understood, the employment of solutions or mixtures of varying consistency as to plasticity, stiffness, or fluidity, depending generally upon the proportion and kind of solvent used to the amount of the original base—acetyl cellulose.

It has been known for many years that camphor and ethyl alcohol in admixture form a solvent for nitrocellulose in the cold or at room temperature and also that camphor can be mixed with the nitrocellulose and that the subsequent addition of ethyl alcohol causes solution or conversion of the nitrocellulose, but the object of my invention was to find substances which, when added to acetyl cellulose, would exert a solvent action upon the cellulose and produce a plastic mass which could be worked in a manner analogous to nitrocellulose-camphor compounds.

I have discovered that acetyl cellulose of the variety which is soluble in acetone can be made into plastic solids by the use of either tetrachlorethyl acetyl cellulose or trichlormethyl acetyl cellulose, or a mixture of the two, in conjunction with ethyl alcohol in substantially equal proportions of the solids and the alcohol and that the solvent will convert the cellulose and render the compound capable of being worked as in the case of the nitrocellulose-camphor plastic art.

As one example of practising my invention, I take 100 parts of an acetyl cellulose of the variety which is soluble in acetone and incorporate it by mixing, grinding, or otherwise, with 35 parts of either tetrachlorethyl

acetanilid or trichlormethyl acetanilid, or a mixture of the two. I then incorporate the mixture with from 40 to 50 parts of ethyl alcohol by stirring and allow the mass to soak or macerate at room temperature in a closed vessel, say, from 12 to 30 hours in order to give good penetration. The mixture is then placed in a steam jacketed mixing machine or a boiling hot water bath (the degree of heat being 100° C.) and after thorough mixing under the influence of heat the resultant mass is then pressed in suitable forms or presses so as to form blocks or cakes while still under the influence of heat, and then after cooling, these blocks or cakes can be cut into sheets or other shapes and subsequently dried or seasoned in the manner analogous to that practised in the nitrocellulose plastic art. Or, if desired, the plastic heated mass can be pressed in heated molds of the desired shape of the final product and subsequently cooled and dried, but the cooling in both cases mentioned above should take place while the heated mass is still under pressure.

It will of course be understood by those skilled in the art that the order of mixing the various ingredients of the compound can be changed if desired and that coloring matters and other inert substances may be incorporated in the compound, and it will also be understood by the operator that slight variations in the proportions of the ingredients named may occur intentionally or designedly, without departing from the spirit of my invention.

Among the chlorinated alkyl acetyl celluloses usable in my process are tetrachlorethyl acetyl cellulose and trichlormethyl acetyl cellulose, both of which when melted are a solvent for acetyl cellulose and which in the presence of ethyl alcohol are a non-solvent for acetyl cellulose at room temperature.

Having thus described my invention, what I claim is:—

1. The process of making acetyl cellulose plastic masses which comprises incorporating an acetone-soluble acetyl cellulose with tetrachlorethyl acetyl cellulose in the presence of a small proportion of ethyl alcohol and heating.
2. The process of making acetyl cellulose plastic masses which comprises incorporating an acetone-soluble acetyl cellulose with a chlorinated alkyl acetyl cellulose in the pres-

ence of a small proportion of ethyl alcohol, and heating, said chlorinated alkyl acetanilid when melted being a solvent for acetyl cellulose and when in the presence of ethyl alcohol being a non-solvent for acetyl cellulose at room temperature.

3. The process of making acetyl cellulose plastic masses which comprises incorporating an acetone-soluble acetyl cellulose with 10 tetrachlorethyl acetanilid in the presence of a small proportion of ethyl alcohol and heating, the proportion of the alcohol being about 1 to 1½ times the acetanilid ingredient.

15 4. The process of making acetyl cellulose plastic masses which comprises incorporating an acetone-soluble acetyl cellulose with a chlorinated alkyl acetanilid in the presence of a small proportion of ethyl alcohol, 20 and heating, said chlorinated alkyl acetanilid when melted being a solvent for acetyl cellulose and when in the presence of ethyl alcohol being a non-solvent for acetyl cellulose at room temperature, the proportion 25 of the alcohol being about 1 to 1½ times the acetanilid ingredient.

5. The process of making acetyl cellulose plastic masses which comprises incorporating an acetone-soluble acetyl cellulose with 30 tetrachlorethyl acetanilid in the presence of

a small proportion of ethyl alcohol and heating, the proportion of the alcohol being about 1 to 1½ times the acetanilid ingredient, and the latter being less than one-half the acetyl cellulose ingredient.

6. The process of making acetyl cellulose plastic masses which comprises incorporating an acetone-soluble acetyl cellulose with a chlorinated alkyl acetanilid in the presence of a small proportion of ethyl alcohol, 40 and heating, said chlorinated alkyl acetanilid when melted being a solvent for acetyl cellulose and when in the presence of ethyl alcohol being a non-solvent for acetyl cellulose at room temperature, the proportion 45 of the alcohol being about 1 to 1½ times the acetanilid ingredient, and the latter being less than one-half the acetyl cellulose ingredient.

7. The process of making acetyl cellulose 50 plastic masses which comprises incorporating an acetone-soluble acetyl cellulose with a chlorinated alkyl acetanilid in the presence of a small proportion of ethyl alcohol and heating.

WILLIAM G. LINDSAY.

Witnesses:

J. E. HINDON HYDE,  
MABEL DENTON.